

Sept. 6, 1938.

K. WÜRSTLIN

2,129,296

SCREEN FOR X-RAY PHOTOGRAPHY

Filed May 7, 1936



Karl Würstlin

INVENTOR

BY *O. Würstlin*

his ATTORNEY

## UNITED STATES PATENT OFFICE

2,129,296

## SCREEN FOR X-RAY PHOTOGRAPHY

Karl Würstlin, Berlin, Germany, assignor to Kali-Chemie Aktiengesellschaft, Berlin, Germany

Application May 7, 1936, Serial No. 78,397  
In Germany May 10, 1935

4 Claims. (Cl. 250—34)

This invention relates to screens for X-ray (Röntgen ray) photography. As is well known, screens are used in making X-ray pictures in order to reduce the time of exposure. The 5 screens generally consist of a sheet of cardboard or Celluloid to the surface of which a fluorescent substance such as calcium tungstate is applied in crystal form and as uniformly as possible by means of a binding agent. The so-called carrier-less screens have also been employed, which consist only of a layer of gelatine containing calcium tungstate.

An object of the invention is to provide a screen with which X-ray photographs of much better 15 sharpness can be obtained than with the known screens, the time of exposure being the same. A further object of the invention is to provide a screen which contains the active layer of calcium tungstate in the form of a mixture of coarse 20 grains and finer grains.

A further object of the invention is to provide a screen having a layer containing fluorescent material in which there are arranged in this active layer between coarser grains of the fluorescent 25 material grains of the same material of considerably smaller diameter and in quantity such that the intermediate spaces between the coarser grains are filled for the most part by the material of finer grain.

30 Further important features and advantages of the invention will be clear from the following description.

It is known that screens containing a layer of calcium tungstate reduce the time of exposure. 35 The use of these screens has, however, the disadvantage that they have an unfavourable effect upon the sharpness of the photographs owing to the occurrence of reflected rays. If the attempt be made to obviate this disadvantage by treating 40 the layer containing the calcium tungstate with a dyestuff or with a light-absorbing medium or by arranging behind the active layer a layer which does not substantially reflect the light emerging from the active layer or by considerably reducing 45 the thickness of the active layer, then, it is true, an improvement in sharpness is obtained; this improvement is, however, only obtained at the expense of an increase in the time of exposure, which may be considerable.

50 It has now been found that the sharpness obtained with the use of a screen can be considerably increased without the time of exposure being simultaneously prolonged by adding to the calcium tungstate used for the manufacture of 55 the known screens or foils a larger or smaller

quantity of a calcium tungstate of very fine grain. The very fine-grained calcium tungstate fills the spaces between the coarser crystals. It is clear that in this way the occurrence of reflected rays is greatly suppressed so that sharper pictures are 5 obtained.

As regards the size of the crystals of the coarse-grained tungstate, they may vary within wide limits. Thus, for example, material of from 4 to 5 or 7 to 8 or 10 $\mu$  can be used. The fine-grained tungstate must possess in comparison with the coarse-grained tungstate a size of grain such that it is adapted substantially to fill up the intervening spaces between the coarser grains. The best results are obtained when the size of 15 grain of the very fine-grained tungstate does not substantially exceed 1 $\mu$ .

The amount of fine-grained tungstate which is added can vary within considerable limits, for example it may amount to about 20 to 25% of the 20 total amount of tungstate. The percentage of very fine-grained tungstate can, however, be considerably higher, but care should be taken if the best results are to be obtained that so much fine-grained tungstate of a size of grain which 25 preferably does not considerably exceed 1 $\mu$  is present that the spaces between the larger crystals are filled as completely as possible. What proportion is most favourable when using a coarser material of a definite size of grain can 30 easily be determined by making a number of comparative exposures.

The invention is illustrated by way of example in the accompanying drawing which shows an elevated view of a screen according to the present 35 invention.

In the drawing 1 is a carrier sheet consisting of cardboard, Celluloid or the like. 2 designates an active layer of calcium tungstate in crystal form glued to the carrier sheet by means of a 40 transparent acetyl cellulose lacquer. According to the present invention the active layer 2 contains calcium tungstate.

The active layer of a screen contains calcium tungstate of a grain size of from 4 to 5 $\mu$  and of a 45 grain size of about 1 $\mu$  in the ratio of 1:1. When a screen of this kind is used for X-ray exposures, photographs are obtained which are in no way inferior as regards sharpness to the pictures obtained with the use of a screen having a dyed 50 active layer. At the same time, however, the time required for exposure is considerably less and amounts to about half the time required when dyed screens are employed.

The symbol " $\mu$ " or "micron" used in the fore- 55

going specification and in the following claims to designate the magnitude of the grain size, signifies 0.001 mm.

I claim:—

- 5 1. A screen for Röntgen ray exposures in which the active layer contains 50% calcium tungstate having a size of grain of from 4 to  $5\mu$  and 50% calcium tungstate consisting of grains of about and not exceeding  $1\mu$  in size.
- 10 2. A screen for Röntgen ray photographic purposes having a layer of fluorescent material, said layer containing 50 to 80% of the fluorescent material in the form of grains having a size of at least  $4\mu$ , and the remaining portion of fluorescent

material consisting of grains not exceeding  $1\mu$  in size.

3. A screen, as claimed in claim 1, in which the said layer contains a sufficient quantity of said smaller grains, to substantially fill the spaces between said coarser grains. 5

4. A screen for Röntgen ray photographic purposes having an active layer of calcium tungstate, said layer containing 50 to 80% of the calcium tungstate in the form of grains having a size 10 between 4 and  $10\mu$ , the remaining portion of the calcium tungstate consisting of grains not greater in size than  $1\mu$ .

KARL WÜRSTLIN.